

## UNITED STATES PATENT OFFICE.

ERNEST F. DIETRICH, OF CHICAGO, ILLINOIS

## PROCESS FOR PLATING METAL ON NONMETALLIC SURFACES.

No Drawing.

Application filed May 20, 1922. Serial No. 582,471.

*To all whom it may concern:*

Be it known that I, ERNEST F. DIETRICH, a citizen of France, and a resident of Chicago, in the county of Cook and State of Illinois, have invented a new and useful Improvement in Processes for Plating Metal on Non-metallic Surfaces, of which the following is a full, clear, and exact description.

10 My invention relates to improvements in the process for plating metal on non-metallic surfaces, such as china, porcelain, glass, or the like, and it consists in the steps hereinafter described and the combinations, 15 constructions, and arrangements herein described and claimed.

An object of my invention is to provide a process of the character described in which metals, such as silver, gold, or nickel, may 20 be permanently deposited on non-metallic surfaces by an electro-plating bath.

A further object of my invention is to provide a process of the character described in which a water impervious glue is employed for supporting a current conducting substance, permitting the deposit of metals thereupon by electro-plating process.

A further object of my invention is to provide a process of the character described in which the metal deposits will not become 30 loosened by heat or moisture.

Other objects and advantages will appear in the following specification, and the novel features of the invention will be particularly pointed out in the appended claims.

In carrying out my invention, I make use of a non-metallic article, such as glass dish or china dish, upon which it is desired to deposit a plating of a metal.

40 I first place a quantity of a good grade of either gelatine or glue in a receptacle containing water and let the gelatine or glue soak thus for at least twenty four hours.

I then place the gelatine or glue over a 45 moderate fire and add thereto 1 part of hydrochloric acid to 10 parts of gelatine. The mixture is then stirred until it is homogeneous and in nearly a fluid state. The proportion of ingredients given are by volume as well as the proportion of ingredients in the remainder of this specification.

I next add 1 part of zinc sulphate and 1 part of acetic acid to keep the mixture in a liquid state. I then add  $\frac{1}{2}$  part of potassium bichromate and  $1\frac{1}{2}$  parts chromic acid which when thoroughly mixed with the foregoing

60 mixture renders the glue insoluble in water and prevents the glue from loosening when brought into contact with acids or alkalies, and forms a cementitious liquid.

I then mix 1 part of the foregoing cementitious mixture with 2 or 3 parts of a good grade of graphite.

65 The mixture or paint so formed may now be painted on the dish by a hand brush or more preferably an air brush. The dish when painted is then placed in the sun to dry or upon a fire until the paint is thoroughly dried.

70 When the paint on the dish has settled after the drying, it is then plated with copper in the following manner:

The electrolyte used is cyanide of soda mixed with copper carbonate, sodium carbonate and water. The anode is pure copper and the cathode the painted portion of the dish. When current is passed through the plating bath in the manner known to those skilled in the art, a film of copper is deposited upon the painted portion of the 80 dish.

75 This copper plating upon the painted portion may then be used as a body upon which other metals, such as silver, gold, or the like, may be plated in the manner known to those skilled in the plating art. Instead of using graphite as the material for mixing with the gelatinous substance in order to conduct the current, I may use any suitable form of metal powder, such as bronze 90 powder. I find that this works equally as well as graphite.

One of the advantages of articles, such as china, dishes, glassware and porcelains having a metal plate thereupon is that the 95 article is rendered stronger by the presence of the metal and yet possess all of the advantages of the materials of which the base of the articles are made.

Another advantage of my process is that the articles may be treated in the manner described at relatively little expense and in a relatively short time.

I claim:

1. The herein described process for plating metal on non-metallic substance which consists in painting the substance with a mixture containing glutinous substance and an electrically conducting material and subsequently plating the painted portion of the 105 substance with a metal in an electro-plating bath.

2. The herein described process for plating metal on a non-metallic substance, which consists in painting the substance with a mixture containing a gelatinous substance, and an electrically conducting material and subsequently plating the painted portion of the substance with a metal in an electro-plating bath. 25
3. The herein described process for plating metal on a non-metallic substance, which consists in painting the substance to be plated with a mixture containing gelatine, potassium bichromate, chromic acid, and graphite and subsequently plating the painted portion of the substance with a metal in an electro-plating bath. 30
4. The herein described process for plating metal on a non-metallic substance, which consists in painting the substance to be plated with a mixture containing glue, potassium bichromate, chromic acid, and graphite and subsequently plating the painted portion of the substance with a metal in an electro-plating bath. 35
5. The herein described process for plating metal on a non-metallic substance, which consists in coating the substance with a mixture containing 10 parts of gelatine,  $\frac{3}{4}$  part of potassium bichromate, and  $1\frac{1}{2}$  part of chromic acid, whereby the gelatine is rendered insoluble in water and subsequently plating the coated portion of said substance with a metal in an electro-plating bath. 40
6. The herein described process for making a current conducting paint which consists in mixing gelatine with water, in adding hydrochloric acid, in stirring the mixture to a homogenous semi-liquid state, and subsequently adding potassium bichromate and chromic acid. 45
7. The herein described process for making current conducting paint which consists in mixing gelatine with water, in adding hydrochloric acid, in stirring the mixture to a homogenous semi-liquid state, and subsequently adding  $\frac{3}{4}$  part potassium bichromate and  $1\frac{1}{2}$  parts of chromic acid. 50

ERNEST F. DIETRICH.